

July 29, 1969

W. HEIMANN ET AL

3,458,379

WINDOW FOR INFRA-RED DETECTORS AND METHOD OF MAKING THE SAME

Filed May 11, 1964

Fig.1



Fig.2



INVENTORS

Walter Heimann

Hans Hoffmann

BY

Michael J. Hinman

*MAH*

**1**

3,458,379

**WINDOW FOR INFRA-RED DETECTORS AND  
METHOD OF MAKING THE SAME**

Walter Heimann, Wiesbaden-Dotzheim, and Hans Hofmann, Wiesbaden, Germany, assignors to Forschungslaboratorium, Prof. Dr. Ing. Walter Heimann, Wiesbaden-Dotzheim, Germany

Filed May 11, 1964, Ser. No. 366,257

Claims priority, application Germany, May 14, 1963,

F 39,733

Int. Cl. B29c 27/00

U.S. Cl. 156—272

6 Claims

**ABSTRACT OF THE DISCLOSURE**

An opening defined by an edge portion of a metal member is hermetically closed by superposing upon the edge portion a substantially plated-shaped body of a material selected from the group consisting of potassium bromide, caesium bromide, caesium iodide and mixed crystals of thallium bromide and thallium iodide and having a melting point below the melting point of the metal member, so as to cover the opening with the plate-shaped body, the latter being supported by the edge portion of the metal member, heating the edge portion of the metal member to the melting temperature of the body so as to melt the portion of the body contacting the thus heated metal edge portion causing downward gravity flow of molten material of the body around the metal edge portion so as to entrain the same and simultaneously lowering of the body into the opening, and reducing the temperature of the metal edge portion to below the melting temperature of the body when the body has been lowered into the opening for a predetermined distance.

The present invention relates to windows for infra-red detectors and to a method of making the same. More particularly, the present invention is concerned with providing an hermetic seal between the window-forming material and the adjacent housing portion.

The materials which form the window panes or windows for vacuum-tight or hermetically closed infra-red detectors generally have a high thermal expansion coefficient, such as for instance, the material known as KRS 5 which is a mixed crystal of thallium-bromide and thallium iodide. Furthermore, these materials for instance, potassium bromide, caesium bromide, caesium iodide, frequently possess only very little mechanical strength. In addition, these materials frequently are hydroscopic.

In view thereof, the connection between such window material and the housing, which connection must form a hermetic seal, is frequently formed of organic compositions such as epoxy resins or of inorganic connecting or binder materials such as silver chloride.

However, it is well known that organic compounds or compositions are not desirable for forming a vacuum-tight seal, because by using organic compositions it is generally not possible to obtain absolute gas-tightness, and it is also generally not possible to obtain the desired degree of mechanical strength. On the other hand, using inorganic materials as the sealing material is undesirable because these sealing materials might react with the crystals forming the window.

It is therefore an object of the present invention to overcome the above discussed difficulties and disadvantages.

It is a further object of the present invention to provide a window for infra-red detectors and a method of making the same which window can be produced in a simple and economical manner, while simultaneously as-

**2**

suring a gas-tight seal of sufficient mechanical strength between the window material and the frame or metal edge of the window opening.

Other objects and advantages of the present invention will become apparent on further reading of the description and of the appended claims.

With the above and other objects in view, the present invention contemplates a window portion of a housing for an infra-red detector comprising, in combination, a metal edge portion defining an opening in the housing, and a substantially plate-shaped member of a material having a melting point lower than the melting point of the metal edge portion entraining the same and completely covering the opening, the member forming an hermetic seal with the entrained edge portion.

The present invention is also concerned with a method of hermetically closing an opening defined by an edge portion of a metal member, comprising the steps of superposing upon the edge portion a substantially plate-shaped body of a material having a melting point below the melting point of the metal member so as to cover the opening with the plate-shaped body, the latter being supported by the edge portion of the metal member, heating the edge portion of the metal member to the melting temperature of the body so as to melt the portion of the body contacting the thus heated metal edge portion causing downward gravity flow of molten material of the body around the metal edge portion so as to entrain the same and simultaneously lowering of the body into the opening, and reducing the temperature of the metal edge portion to below the melting temperature of the body when the body has been lowered into the opening for a predetermined distance.

Thus, according to the present invention, a suitable window pane material is placed on top of the opening which is to be closed so that it will rest on the thin metal edge which defines such opening. The window pane material will have dimensions which are somewhat larger than the opening which is to be closed so that an annular edge portion of the window pane material will rest on the annular edge portion of the metal housing which defines the window opening.

Suitable window pane materials includes crystals of potassium bromide, caesium bromide, caesium iodide, and mixed crystals of thallium bromide and thallium iodide known as KRS5.

The metal edge portion upon which the peripheral portion of the window pane crystal is superposed, is then heated to at least the melting point of the window pane material. This can be advantageously accomplished by means of a high frequency induction coil, in other words, by induction heating. As soon as the metal-supported peripheral portion of the window pane crystal starts to melt, the crystal will start by gravity to be lowered into the window opening. When the crystal has penetrated the window opening to the desired depth, heating of the metal edge portion is interrupted, and it is thereby achieved that the temperature of the metal edge portion and of the portion of the crystal in contact therewith, will quickly drop below the melting point of the material of the crystal and, upon such solidification, the crystal will not penetrate further downwardly into the window opening.

According to the present method, the window material will melt only in the immediate vicinity of the supporting annular metal edge portion which defines the opening which is to be closed. The major portion of the crystal, i.e., the entire crystal with the exception of the peripheral portion thereof, will remain solid and unharmed. The thus molten peripheral portion of the crystal will, upon cooling and solidification, form a hermetic seal with the metal edge.

Since the metal edge is formed of a very thin metal sheet, the tension stresses which will occur upon cooling of the window pane material and the metal, due to the different rate of reduction in the length thereof upon cooling, will be easily taken up. It is important that any remaining tension will be directed thereby in radial symmetry towards the center of the window pane material. These residual tensions will be easily taken up by the crystal forming the window pane, since they result only in subjecting the window pane material to a slight degree of pressure.

It is possible, according to the present invention, to close openings in flat metal sheets, as well as the end portion of tubular members.

In order to avoid too deep a penetration of the window material into the metal or of the metal edge into the window material, it is preferred according to the present invention, to place underneath the opening a flat sheet, or underneath the end portion of a tube which is to be closed according to the present invention, a member which will support the window material when it has penetrated to the desired depth so that the window material will be prevented from further downward movement once it has reached the supporting or stopping member.

The heating of the metal edge which defines the window which is to be closed can be carried out in any desired manner, however, it is preferred to carry out this localized heating by means of a high frequency induction coil. The metal edge portion which forms or defines the opening or window which is to be closed according to the present invention, should consist of one of the metals which are suitable for forming a hermetic seal with molten material, preferably silver. The thickness of the metal edge portion preferably will be between 0.05 and 0.1 millimeter.

The crystal which is to form the window is placed on the opening preferably so that it will extend outwardly of the window opening and will be supported by the metal edge portion along a peripheral edge of the crystal having a width of between about 0.5 and 1.0 millimeter. The overall dimensions, i.e., the length and width, of such crystal window pane may be of the magnitude of about 10 millimeters.

The novel features which are considered as characteristic for the invention are set forth in particular in the appended claims. The invention itself, however, both as to its construction and its method of operation, together with additional objects and advantages thereof, will be best understood from the following description of specific embodiments when read in connection with the accompanying drawings, in which:

FIG. 1 is a cross-sectional somewhat diagrammatic elevational view of an arrangement for closing an opening defined by the annular edge of a tubular housing member; and

FIG. 2 is a somewhat diagrammatic, elevational view in cross section illustrating the closing of a window opening in a flat metal sheet member of the housing.

Referring now to the drawing, in both figures reference numeral 1 denotes the crystal which serves for closing the window, while reference numerals 2 and 22 respectively indicate the metal edge portion defining the window opening which is to be closed. Members 3 and 23 respectively are arranged underneath the window opening, according to FIG. 1 outwardly of the tubular member 2, and according to FIG. 2 below the flat metal sheet 22, for supporting window material 1 as soon as the same has penetrated the window opening to the desired depth.

Heating of the edge portion 5 is carried out by means of induction coil 4.

As soon as metal edge portion 5 will be thus heated to the melting temperature of the window pane material 1, the window pane material will penetrate the window edge 5, and will slowly move downwardly by gravity until it is supported by supporting member 3. At this moment,

i.e. as soon as contact has been established between window material 1 and supporting member 3, heating is interrupted and upon cooling and solidification of the molten peripheral portion of window material 1, an hermetically sealing bond between window material 1 and metal edge portion 2 will be established.

In order to achieve, according to the embodiment illustrated in FIG. 2, that the molten portion of material 1 will embed the annular edge of flat sheet 22, which edge portion defines the window, it has been found advantageous to give to the upper face of the stopping member 23 a shape and size somewhat larger than that of the window, and to have the peripheral edge of the upper face of holding member 23 extending upwardly as shown in FIG. 2.

It will be understood that each of the elements described above, or two or more together, may also find a useful application in other types of hermetic sealing arrangements differing from the types described above.

While the invention has been illustrated and described as embodied in a window portion of a housing for an infra-red detector, it is not intended to be limited to the details shown, since various modifications and structural changes may be made without departing in any way from the spirit of the present invention.

Without further analysis, the foregoing will so fully reveal the gist of the present invention that others can by applying current knowledge readily adapt it for various applications without omitting features that, from the standpoint of prior art, fairly constitute essential characteristics of the generic or specific aspects of this invention and, therefore, such adaptations should and are intended to be comprehended within the meaning and range of equivalence of the following claims.

What is claimed as new and desired to be secured by Letters Patent is:

1. A method of hermetically closing an opening defined by an edge portion of a metal member, comprising the steps of superposing upon said edge portions a substantially plate-shaped body of a material selected from the group consisting of potassium bromide, caesium bromide, caesium iodide and mixed crystals of thallium bromide and thallium iodide and having a melting point below the melting point of said metal member so as to cover said opening with said plate-shaped body, the latter being supported by said edge portion of said metal member; heating said edge portion of said metal member to the melting temperature of said body so as to melt the portion of said body contacting the thus heated metal edge portion causing downward gravity flow of molten material of said body around said metal edge portion so as to entrain the same and simultaneously lowering of said body into said opening; and reducing the temperature of said metal edge portion to below the melting temperature of said body when said body has been lowered into said opening for a predetermined distance.

2. A method of hermetically closing an opening forming a window portion of a housing for an infra-red detector and being defined by an annular edge portion of a metal tube, comprising the steps of superposing upon said edge portion a substantially plate-shaped body of material selected from the group consisting of potassium bromide, caesium bromide, caesium iodide and mixed crystals of thallium bromide and thallium iodide and having a melting point below the melting point of said metal member so as to cover said opening with said plate-shaped body, the latter being supported by said edge portion of said metal member; heating said edge portion of said metal member to the melting temperature of said body so as to melt the portion of said body contacting the thus heated metal edge portion causing downward gravity flow of molten material of said body around said metal edge portion so as to entrain the same and simultaneously lowering of said body into said opening; and reducing the temperature of said metal edge portion to

below the melting temperature of said body when said body has been lowered into said opening for a predetermined distance.

3. A method of hermetically closing an opening forming a window portion of a housing for an infra-red detector and being defined by an annular edge portion of a substantially flat sheet metal member, comprising the steps of superposing upon said edge portion a substantially plate-shaped body of a material selected from the group consisting of potassium bromide, caesium bromide, caesium iodide and mixed crystals of thallium bromide and thallium iodide and having a melting point below the melting point of said metal member so as to cover said opening with said plate-shaped body, the latter being supported by said edge portion of said metal member; heating said edge portion of said metal member to the melting temperature of said body so as to melt the portion of said body contacting the thus heated metal edge portion causing downward gravity flow of molten material of said body around said metal edge portion so as to entrain the same and simultaneously lowering of said body into said opening; and reducing the temperature of said metal edge portion to below the melting temperature of said body when said body has been lowered into said opening for a predetermined distance.

4. A method of hermetically closing an opening forming a window portion of a housing for an infra-red detector and being defined by an edge portion of a metal member, comprising the steps of superposing upon said edge portion a substantially plate-shaped body of a material selected from the group consisting of potassium bromide, caesium bromide, caesium iodide and mixed crystals of thallium bromide and thallium iodide and having a melting point below the melting point of said metal member so as to cover said opening with said plate-shaped body, the latter being supported by said edge portion of said metal member; heating said edge portion of said metal member to the melting temperature of said body so as to melt the portion of said body contacting the thus heated metal edge portion causing downward gravity flow of molten material of said body around said metal edge portion so as to entrain the same and simultaneously lowering of said body into said opening; and preventing further downward movement of said body and reducing the temperature of said metal edge portion to below the melting temperature of said body when said body has been lowered into said opening for a predetermined distance.

5. A method of hermetically closing an opening defined by an edge portion of a metal member consisting essentially of silver, comprising the steps of superposing upon said edge portion a substantially plate-shaped crys-

talline body of a material being selected from the group consisting of potassium bromide, caesium bromide, caesium iodide and mixed crystals of thallium bromide and thallium iodide, and having a melting point below the melting point of said metal member so as to cover said opening with said plate-shaped body, the latter being supported by said edge portion of said metal member; heating said edge portion of said metal member to the melting temperature of said body so as to melt the portion of said body contacting the thus heated metal edge portion causing downward gravity flow of molten material of said body around said metal edge portion so as to entrain the same and simultaneously lowering of said body into said opening; and reducing the temperature of said metal edge portion to below the melting temperature of said body when said body has been lowered into said opening for a predetermined distance.

6. A method of hermetically closing an opening defined by an edge portion of a metal member, comprising the steps of superposing upon said edge portion a substantially plate-shaped body of a material selected from the group consisting of potassium bromide, caesium bromide, caesium iodide and mixed crystals of thallium bromide and thallium iodide and having a melting point below the melting point of said metal member so as to cover said opening with said plate-shaped body, the latter being supported by said edge portion of said metal member; induction heating said edge portion of said metal member to at least the melting temperature of said body so as to melt the portion of said body contacting the thus heated metal edge portion causing downward gravity flow of molten material of said body around said metal edge portion so as to entrain the same and simultaneously lowering of said body into said opening; and reducing the temperature of said metal edge portion to below the melting temperature of said body when said body has been lowered into said opening for a predetermined distance.

#### References Cited

##### UNITED STATES PATENTS

|           |         |                 |       |             |
|-----------|---------|-----------------|-------|-------------|
| 2,419,049 | 4/1947  | Alpert          | ----- | 287—189.365 |
| 2,542,702 | 2/1951  | Prow            | ----- | 156—273 XR  |
| 2,649,392 | 8/1953  | Marshall        | ----- | 156—273 XR  |
| 2,744,592 | 5/1956  | Remond          | ----- | 287—189.365 |
| 3,220,815 | 11/1965 | McMillan et al. | ----- | 65—32       |

EARL M. BERGERT, Primary Examiner

G. W. MOXON II, Assistant Examiner

U.S. Cl. X.R.

156—303.1